

C. G. MUENCH.

## THERMO NON-CONDUCTOR.

APPLICATION FILED MAR. 7, 1913. RENEWED JAN. 30, 1915.

1,153,512.

Patented Sept. 14, 1915.



Witnesses.

St. Fischer

S. L. Waschenbergs

Inventor:

Carl G. Muench

By: J. Bradbury  
Attorney.

# UNITED STATES PATENT OFFICE.

CARL G. MUENCH, OF ST. PAUL, MINNESOTA.

## THERMO NON-CONDUCTOR.

1,153,512.

Specification of Letters Patent. Patented Sept. 14, 1915.

Application filed March 7, 1913, Serial No. 752,614. Renewed January 30, 1915. Serial No. 5,305.

To all whom it may concern:

Be it known that I, CARL G. MUENCH, a citizen of the United States, residing at St. Paul, in the county of Ramsey and State of Minnesota, have invented a new and useful Improvement in Thermo Non-Conductors, of which the following is a specification.

My invention relates to a new and useful 10 thermo non-conductor to be used for cold storage buildings, refrigerator cars, refrigerators, heater cars, fireless cookers, houses, etc., and consists mainly of large felted sheets, slabs, blocks, tubes and other shapes 15 made of any size and thickness from coarse long wood fibers. The long wood fibers used in my insulating felt are obtained by screening ordinary wood pulp as it comes from the cookers and grinders and using the fine pulp 20 for paper and other purposes and the residue of coarse long and short fibers for my insulation. In other words I use what is known as pulp screenings or tailings, which is at the present time useless, has no value 25 and is only refuse. By using this waste material I produce a very inexpensive and efficient non-conducting felt which is more effective and less expensive to produce than any non-conducting material in use at the 30 present time.

My sheet non-conductor is made by flowing a thin mixture of coarse long and short wood fibers and water upon an endless moving screen passing under a suitable evener 35 said mixture draining and felting as it travels and passing between progressive pressing devices which express moisture and reduce the mixture to a sheet of desired thickness. The sheet is cut into lengths or 40 slabs and the pieces placed in a kiln to dry. The blocks or other shapes are made by casting in a form of the desired shape, pressing slightly and then drying. The sheets or blocks are extremely light, and tough having 45 great tensile strength and containing countless air cells, thus producing an ideal non-conductor having a specific gravity of only fifteen to twenty one-hundredths. The sheets and slabs are also flexible and therefore 50 well adapted for structural purposes. My thermal insulation made of long and short wood fibers can also have a small amount of flax, jute or hemp fiber either singly or together incorporated in it before felting to give it even greater tensile strength without impairing its quality as a

non-conductor. A small percentage of ammonium or other salts or other suitable material can be added to the mixture of long and short wood fibers and water before felting to render the finished product uncom- 60 bustible. By applying a thin coating of hot paraffin wax, paraffin oil, wax tailings or the like to my non-conductor before it is placed in the kiln it will be rendered water proof. 65 As the moisture leaves the felt the fluid oil or wax is drawn through by capillary attraction so that every fiber is permeated and water proofed.

I am aware that ordinary short fiber wood 70 pulp mixed with plaster of Paris, hair, infusorial earth, straw and cork has been proposed for insulation, but this has never been a commercial success. In these mixtures the materials are made into a plastic form and 75 then applied or molded into the desired shape and allowed to dry resulting in a hard rigid material with very little tensile strength. Sheets made of any of these mixtures the size and thickness which are necessary 80 for practical purposes cannot be handled without breaking and are therefore impracticable. The materials mentioned in these mixtures are also too expensive for commercial purposes. My thermal insulation 85 is totally different because instead of being molded, it is felted, that is the long and short wood fibers and water are mixed, so that they are in a thin fluid state, and are then flowed on a screen apron through 90 which the water drains, leaving a thick felted or matted layer of long and short wood fibers which when slightly pressed and dried produces a strong tough sheet, which cannot be produced with ordinary wood pulp. In 95 producing sheets of my improved non-conductor a felting machine is employed, one form of structure being illustrated in the accompanying drawing which forms part of this specification.

The term "long and short wood fibers" as used in this specification and the claims following is relative in so far as related to wood fiber as appearing in the tailings received from a pulp mill, but all of such fibers are 100 short as compared with the fibers found in flax, jute and hemp or in strips or shavings of material such as have been heretofore used in the manufacture of insulating board and I do not claim such structure except in relation to tailings received from a pulp mill. 110

In this drawing, Figure 1 is a longitudi-

nal section of the machine; Fig. 2 is a cross section of the machine taken on the line X—X of Fig. 1, and Fig. 3 is a detail illustrating part of the driving mechanism.

5 In this drawing, A represents a screen endless apron, the upper lap of which moves forward over the bed 2, said apron passing around the idle pulley 3, and the drive pulley 4. The upper lap of the belt and the 10 bed of the machine incline upwardly from the idle pulley toward the drive pulley. The lower end of the lap receives a thin solution or mixture of long wood fibers and water from the tank B, said solution being 15 spread evenly upon the surface of the apron, an evener 5 being employed to assist in spreading the mixture evenly and said evener being revolved and said apron driven in the direction of the arrows indicated in 20 Fig. 1. After the wood pulp mixture C advances with the apron, the water gradually drains through the apron, the thickness of the mixture gradually reducing as the belt advances. The upper lap of the apron near 25 its upper end passes between progressive pairs of pressing rollers, D, E and F, which serve to press the felted or matted layer of long coarse wood fibers step by step until ultimately the liquid in the lap is expressed 30 leaving a sheet of non-conducting material in moist condition, which is ejected from the apron upon a traveling conveyer G, said conveyer carrying the sheet forward over the idle rollers H on to trays such as I.

35 Each tray I is placed on a conveyer 6, which travels in the direction of the arrows shown in Fig. 1, and serves to move the tray forward so as to catch and conduct the sheet of non-conducting material while it is 40 egressing from the machine. When the successive trays I receive the strip of non-conducting material, said strip is cut by hand into short lengths or slabs which are carried away by an attendant on the trays 45 and placed in a drying kiln. After the kiln has been filled with the loaded trays and the sheets or slabs of non-conducting material on the trays dried or baked, strong tough sheets or slabs of non-conducting

material are completed in readiness for 50 commercial use. Said finished sheets or slabs are of sufficient strength to permit being fastened upon the walls of refrigerator cars without disintegration due to jolting and vibration.

55

The apron A, compression rollers D, E and F, and conveyer belts G and I are advanced at equal surface speed by any suitable mechanism, the drawing illustrating a train of gears J operated by the drive pulley 7 by which the speed of operation is reduced so that the actuated parts move at very slow speed. At the sides of the upper lap of the belt A, deckels 10 are provided which serve as guards, to prevent the mixture when in fluid state from running over the sides of the belt and to produce a sheet of material of even width having smooth regular side edges. Below the apron A, a tank 8 is placed having a drain 9, said tank 70 serving to catch any drip from the apron which is expressed from the pulp mixture.

65

The term "tailings" as used in this specification and the claims following is intended to include the product commonly known as 75 screenings which are the waste product of a pulp mill.

80

Having described my invention, what I claim as new and desire to protect by Letters Patent is:—

1. A thermal non-conductor composed of wood pulp tailings felted into a light, spongy sheet, pressed slightly and dried.
2. A thermal non-conductor composed of wood pulp tailings felted into a sheet or 85 other shape, fire proofed, pressed slightly and dried.
3. A thermal non-conductor composed of wood pulp tailings, water-proofed, felted into a sheet or other shape, pressed slightly 90 and dried.

In testimony whereof, I have signed my name to this specification in the presence of two subscribing witnesses.

CARL G. MUENCH.

Witnesses:

A. L. FISCHER,  
F. G. BRADBURY.